

# UNITED STATES PATENT OFFICE.

JOHN E. FOWLER, OF YOUNGSTOWN, OHIO. ASSIGNOR OF ONE-HALF TO  
HOWARD H. BECK, OF YOUNGSTOWN, OHIO.

## CASTING BRASS OR OTHER COPPER ALLOYS INTO METALLIC MOLDS.

No. 826,157.

Specification of Letters Patent.

Patented July 17, 1906.

Application filed September 5, 1905. Serial No. 276,966.

*To all whom it may concern:*

Be it known that I, JOHN E. FOWLER, a citizen of the United States, and a resident of Youngstown, county of Mahoning, and State of Ohio, have invented a new and useful Improvement in Processes of Casting Brass or other Copper Alloys into a Metallic Mold, of which the following is a specification, the principle of the invention being herein explained and the best mode in which I have contemplated applying that principle, so as to distinguish it from other inventions.

My invention relates to processes of casting molten metal into a metallic mold, and particularly to casting brass or other copper alloys into a steel mold.

My said invention consists of that part or steps of such process which involves the treatment of the interior of the mold for the reception of the molten brass or other copper alloy, hereinafter fully described, and particularly set forth in the claims.

The following description sets forth in detail one mode of carrying out the invention, such disclosed mode constituting but one of various ways in which the principle of the invention may be used.

In the application of my improved process I treat the smooth interior of an iron or steel, preferably iron, mold in such a manner as to prevent any uniting or penetrating action from taking place between the molten metal and the iron of the mold, thereby preventing the casting from uniting with the mold and permitting its ready separation therefrom after the casting is cool and ready for removal. I effect this result by producing a covering of borates on the interior of the mold, and this is done by treating the interior mold-surface to the action of a boron compound in dilute liquid solution, such as will produce such borates. This solution may be applied by dipping, washing, or in any desired manner, and I have found the use of a dilute liquid solution of boracic acid to be the most practical and advantageous for effecting the required action. I have found that this boracic-acid solution when so applied has a great penetrating effect upon the iron or steel mold and most thoroughly af-

fects all such particles of the mold as might otherwise be reached by the molten metal. A resulting formation of borate compounds is effected on the mold and in the interstices thereof. The chemical affinities of the boracic acid are therefore satisfied, and said borates do not combine chemically or amalgamate with the brass or other copper alloys, are indestructible by heat as well as insoluble, and form an effectual barrier to the union of the mold with the molten metal. The liquid form of the applied boracic acid permits a comparatively very small amount thereof to be used, so that the interior of the mold preserves its smooth hard finish and imparts the same physical characteristics of smoothness to the casting. In this manner any number of castings may be made in the same mold. The castings are comparatively smooth and require a minimum application of further labor of machining and finishing.

Having thus described my invention in detail, that which I particularly point out and distinctly claim as my invention is—

1. In the process of casting brass or other similar copper alloys into a metallic mold, that step which consists in subjecting the interior of the mold to the chemical action of a compound of boron such as will form borates.

2. In the process of casting brass or other similar copper alloys into a metallic mold, that step which consists in subjecting the interior of the mold to the chemical action of boracic acid.

3. In the process of casting brass or similar copper alloys into a metallic mold, that step which consists in subjecting the interior of the mold to the chemical action of boracic acid in liquid solution.

4. In the process of casting brass or similar copper alloys into a metallic mold, that step which consists in subjecting the interior of the mold to the chemical action of boracic acid in dilute liquid solution.

Signed by me this 26th day of August, 95  
1905.

JOHN E. FOWLER.

Attest:

FRANK L. OESCH,  
W. B. RANDOLPH.